# EUROPEAN PATENT APPLICATION

(11) **EP 0 997 545 A1**
(43) Date of publication of application: **03.05.2000**
(21) Application number: 99121491.7
(22) Date of filing: 28.10.1999
(51) Int. Cl.: C22C 21/00, C22F 1/04, C25D 11/04

(54) **Ornamental aluminum alloy member and process for producing the same**

(30) Priority: 30.10.1998 JP 31138398
(71) Applicant: Casio Computer Co., Ltd., Shibuya-ku, Tokyo (JP)
(72) Inventor: Hashikura, Manabu, c/o Itami Works, Itami-shi, Hyogo-ken (JP); Hattori, Hisao, c/o Itami Works, Itami-shi, Hyogo-ken (JP); Kaji, Toshihiko, c/o Itami Works, Itami-shi, Hyogo-ken (JP); Takeda, Yoshinobu, c/o Itami Works, Itami-shi, Hyogo-ken (JP); Yatabe, Mitsunobu, c/o Hamura R&D Center, Hamura-shi, Tokyo 205-8555 (JP); Kido, Yukio, c/o Hamura R&D Center, Hamura-shi, Tokyo 205-8555 (JP)
(74) Representative: Grünecker, Kinkeldey, Stockmair & Schwanhäusser Anwaltssozietät

(57) **Abstract**

An ornamental aluminum alloy member (10) has a substrate (1) made of an aluminum alloy, and an anodic oxidation film (2) formed on a surface of the substrate. The aluminum alloy forming the substrate (1) contains from 0.1% to 3% by weight of Zr, from 0.1% to 15% by weight of Mischmetal (Mm), from 0.1% to 5% by weight of Mg, optionally from 0.1% to 5% by weight of at least one metal element selected from the group consisting of Mo, W, Nb, Ag and Ta, and the balance of Al.

## Description

The present invention relates to an ornamental aluminum alloy member, and a process for producing the same.

In the prior art of this field, a rod or a plate made of a molten aluminum alloy has been cold-molded or warm- or hot-molded into a desired shape and then the molded product has been subjected to surface treatment by anodic oxidation.

It is recognized in the art that the mechanical strength of molten aluminum is relatively low. In order to enhance the mechanical strength of the molten aluminum, Mg (magnesium), an additive element or elements such as Cu (copper), Si (silicon), and Zn (zinc) are added to the aluminum. The resultant aluminum alloy is surface treated by anodic oxidation or low-temperature anodic oxidation (hard anodization treatment) so as to harden its surface. The so treated aluminum alloy is used as an ornamental members such as exterior parts for watches.

As described above, conventionally, a molten aluminum alloy containing an additive element such as Mg, Cu, Si and Zn has been often used in view of the strength in the range of use temperature of exterior parts, e.g., for watches. However, since the molten aluminum contains these elements, the mechanical strength in the range of working temperature of the aluminum alloy is also relatively enhanced, resulting in that it is relatively difficult to cold-mold or hot-mold the aluminum alloy. In particular, there remarkably occur deformation of the metal crystals due to plastic deformation at the time of cold-molding, or warm- or hot-molding, and increase in the internal stress, that is, work hardening. Therefore, the cold-moldability, or warm- or hot-moldability becomes poor. Thus, when the aluminum alloy is molded into a complicated shape, stepwise molding is necessary for obtaining such a complicated final shape, leading to high costs.

The molded aluminum alloy is subjected to anodization to provide finished exterior parts for, e.g., watches, after subjected to optional working on lathe or drilling working, followed by buffing. However, the aluminum alloy before the anodic oxidation, that is, the original texture of the aluminum alloy is relatively low in its surface hardness.

Specifically, the surface hardness Hv would be at most 100. This is because the inventors of the present invention have cold-molded the aluminum alloy three times and measured the surface hardness Hv of the molded product according to JIS A5052-O to find that the surface hardness Hv was about 70.

Since the prior art aluminum alloy has a low surface hardness as described above, the alloy is very liable to be injured and care must be sufficiently taken in handling thereof. When the alloy is industrially mass-produced, it has been necessary to account for a certain measure of decrease in the yield.

Further, by applying anodic oxidation or low-temperature anodic oxidation to the surface of the above-mentioned molded product, corrosion resistance thereof is ensured and further abrasion resistance is ensured due to the hardening of its surface. In general, however, the thickness of films produced by anodic oxidation or low-temperature anodic oxidation is at most only about 20 µm. Because of this fact and the above-mentioned relative low hardness of the original texture of the aluminum alloy, the anodized alloy is liable to be injured by external force when used as external parts for watches.

Accordingly, an object of the present invention is to provide an ornamental aluminum alloy member which can be easily molded into a complicated shape and is high in the hardness of its aluminum alloy texture, as well as a process for producing the same.

Another object of the present invention is to provide an ornamental aluminum alloy member whose aluminum alloy texture has high hardness and whose anodic oxidation film is transparent and colorless or is pale in color, such as off-white or silver white.

According to a first aspect of the present invention, there is provided an ornamental aluminum alloy member comprising a substrate made of an aluminum alloy containing from 0.1% to 3% by weight of Zr; from 0.1% to 15% by weight of Mischmetal (hereinafter abbreviated as Mm), from 0.1% to 5% by weight of Mg and the balance of Al; and an anodic oxidation film formed on a surface of the substrate.

According to a second aspect of the present invention, there is provided an ornamental aluminum alloy member comprising a substrate made of an aluminum alloy and an anodic oxidation film formed on the substrate, wherein the substrate has a hardness HRB of from 50 to 100, and the anodic oxidation film has a lightness of 50 or more.

Further, according to the present invention, there is provided a process for producing an ornamental aluminum alloy member, comprising the steps of: (a) forming a molded body made of an aluminum alloy containing from 0.1% to 3% by weight of Zr, from 0.1% to 15% by weight of Mm, from 0.1% to 5% by weight of Mg, and the balance of Al; (b) heating the molded body up to a temperature of from 200°C to 600°C under the condition of a temperature-raising rate of 2°C/second or more; (c) working the heated molded body; and (d) subjecting the worked molded body to anodic oxidation treatment. Usually, the molded body is heated up to 200°C to 600°C, starting from room (ambient) temperature.

This summary of the invention does not necessarily describe all necessary features so that the invention may also be a sub-combination of these described features.

The invention can be more fully under stood from the following detailed description when taken in conjunction with the accompanying drawings, in which:
FIG. 1 is a partial cross sectional view schematically illustrating a structure of a wrist watch case, as an example of the ornamental aluminum alloy member according to the present invention;
FIG. 2 is a view illustrating a first step in a process for producing the case illustrated in FIG. 1;
FIG. 3 is a view illustrating a second step in a process for producing the case illustrated in FIG. 1;
FIG. 4 is a view illustrating a third step in a process for producing the case illustrated in FIG. 1;
FIG. 5 is a view illustrating a fourth step in a process for producing the case illustrated in FIG. 1;
FIG. 6 is a view illustrating a fifth step in a process for producing the case illustrated in FIG. 1;
FIG. 7 is a view illustrating a sixth step in a process for producing the case illustrated in FIG. 1;
FIG. 8 is a view illustrating a seventh step in a process for producing the case illustrated in FIG. 1; and
FIG. 9 is a view illustrating an eighth step in a process for producing the case illustrated in FIG. 1.

The inventors have conducted extensive studies and found a composition of an aluminum alloy which can be easily molded into a complicated shape and can be improved in the hardness of its original aluminum alloy texture.

Specifically, the present invention provides an ornamental aluminum alloy member, comprising: a substrate made of an aluminum alloy comprising from 0.1% to 3% by weight of Zr, from 0.1% to 15% by weight of Mm, from 0.1% to 5% by weight of Mg, and the balance of Al; and an anodic oxidation film formed on a surface of the substrate.

The aluminum alloy having the above composition is lowered in the strength at the working-temperatures and thus its molding into a complicated shape becomes easy. Therefore, the number of molding times for obtaining a final shape can be made less than that in the prior art, so that working costs can be reduced.

Moreover, the aluminum alloy of the invention has an improved hardness, so that the aluminum alloy member is prevented from being injured at the time of handling before anodic oxidation. Even if the members are industrially mass-produced, the yield thereof can be improved more than in the prior art. Since the hardness of the aluminum alloy of the invention is improved, the aluminum alloy member is unlikely to be injured even if the member receives external force after the formation of the anodic oxidation film.

In addition, the inventors have found that in the case of forming an anodic oxidation film on the substrate of the aluminum alloy having the above-mentioned composition, the anodic oxidation film can be made transparent and colorless, off-white or silver white. As a result, in the case of coloring the anodic oxidation film, a desired color can be realized without being affected by the original color of the anodic oxidation film. Therefore, the aluminum alloy member of the present invention is very suitable for ornaments for which a delicate color tone is required.

The following will describe the contents of the additive elements.

Zr has such a function that addition of a small amount thereof makes the crystal grain size of aluminum small to enhance the hardness of the aluminum alloy. However, if Zr forms supersaturated solid-solution at the time of rapid solidification and remains solid-solution after hot-working, an anodic oxidation film which will be produced by anodic oxidation of the aluminum alloy will exhibit a dark color. Thus, the anodic oxidation film can be made transparent and colorless, off-white, or silver white by causing Zr not to form solid-solution and precipitating Zr in the form of an intermetallic compound formed with aluminum.

The Zr content in the aluminum alloy of the invention is set in the range of from 0.1% to 3% by weight. If the Zr content is less than 0.1% by weight, the effect of the addition of Zr cannot be obtained. If the Zr content is more than 3% by weight, the Al-Zr based intermetallic compound grows large so that the anodic oxidation film exhibits a dark color.

In order to obtain better property, the Zr content is preferably from 1.5% to 2.5% by weight.

Mm has such a function that addition of a small amount thereof causes an intermetallic compound having high hardness to be precipitated in a large amount to enhance the hardness of the aluminum alloy. However, if the grains of the precipitated intermetallic compound are large, an anodic oxidation film which will be produced by anodic oxidation of the aluminum alloy will exhibit a dark color. Thus, the color of the anodic oxidation film can be made off-white by making the grains of the precipitated intermetallic compound small.

The Mm content of the aluminum alloy of the invention is set in the range of from 0.1% to 15% by weight. If the Mm content is less than 0.1% by weight, the effect of the addition of Mm cannot be obtained. If the Mm content is more than 15% by weight, the intermetallic compound grows large so that the anodic oxidation film exhibits a dark color.

In order to obtain better property, the Mm content is preferably from 4.0% to 5.0% by weight.

Mg has such a function that it forms supersaturated solid-solution in a large amount into α-aluminum to enhance the hardness.

The Mg content of the aluminum alloy of the invention is in the range of from 0.1% to 5% by weight. If the Mg content is less than 0.1% by weight, the effect of the addition of Mg cannot be obtained. If the Mg content is more than 5% by weight, the anodic oxidation film exhibits a dark color.

In order to obtain better property, the Mg content is preferably from 4.0% to 5.0% by weight.

If the aluminum alloy having the above-mentioned composition is hot-molded and subsequently its surface is polished by buffing or the like, metallic gloss can easily be obtained on the surface of the aluminum alloy.

In the present invention, preferably, the substrate aluminum alloy further contains at least one metal element selected from the group consisting of Mo, W, Nb, Ag and Ta, in an amount of from 0.1% to 5% by weight.

Mo, W, Nb, Ag and Ta have such a function that addition of a small amount thereof causes an intermetallic compound having high hardness to be precipitated in a large amount to enhance the hardness of the aluminum alloy. However, if the grains of the precipitated intermetallic compound are large, an anodic oxidation film which will be produced by anodic oxidation of the aluminum alloy will exhibit a dark color. Thus, the anodic oxidation film can be made a light color tone by making the grains of the precipitated intermetallic compound small.

These additional metal elements are contained in an amount of from 0.1% to 5% by weight as described above. If the content of these elements is less than 0.1% by weight, the effect of the addition of these elements cannot be obtained. If the content of these elements is more than 5% by weight, the precipitated intermetallic compound grows large so that the anodic oxidation film exhibits a dark color.

As described above, the inventors have found that the composition according to the first aspect makes the hardness of the substrate high and makes the anodic oxidation film transparent and colorless, off-white or silver white. More specifically, the substrate made of the aluminum alloy of the present invention as described above may have a hardness HRB (B scale of Rockwell hardness) of from 50 to 100 and the anodic oxidation film may have a lightness (L*) of 50 or more

Thus, according to a second aspect, the present invention provides an ornamental aluminum alloy member comprises a substrate comprising an aluminum alloy, and an anodic oxidation film formed on a surface of the substrate, wherein the substrates has a hardness HRB (B scale of Rockwell hardness) of from 50 to 100 and the anodic oxidation film has a lightness (L*) of 50 or more.

According to the second aspect of the present invention, a hardness HRB is from 50 to 100. Thus, the percentage of inferior products, which are injured in a producing process, can be made far smaller than in the case of conventional molten aluminum alloy according to, e.g., JIS A5052. Further, the lightness (L*) of the anodic oxidation film is 50 or more. Thus, a desired color can be realized without being affected by the original color tone of the anodic oxidation.

The lightness (L*) in this context is lightness in the $\text{L*a*b*}$ color specification system defined in JIS Z8729, and is spectroscopically measured by means of a chromaticity meter. A light source used in the measurement is D65 (International Illumination Committee, ISO standard light), the color temperature of which is 6504K.

The hardness of the substrate is set in the range of from 50 to 100 according to the second aspect of the present invention. If the hardness is less than 50, the aluminum alloy member is liable to be injured. If the hardness is more than 100, its limit upsetting ratio and elongation at room temperature (20°C), as will be described later, decrease.

In the present invention, the electric conductivity of the substrate is preferably 20% IACS or more.

The inventors have found that as the electric conductivity of the substrate is higher, the solid-solutioned amount of the substrate elements into the anodic oxidation film is less so that the color of the anodic oxidation film becomes colorless or lighter, and that the electric conductivity of the substrate must be 20% IACS or more in order that the anodic oxidation film becomes colorless or a light color tone. Moreover, the inventors have found that the electric conductivity of the substrate in the aluminum alloy member of the present invention can become 20% IACS or more. Since the electric conductivity of the substrate in the aluminum alloy member of the present invention becomes 20% IACS or more, the anodic oxidation film becomes colorless or a light color tone. Besides, the present invention can find application where high electric conductivity is required for the substrate.

In the second aspect, too, the anodic oxidation film is preferably transparent and colorless, off-white, or silver white.

Thus, the aluminum alloy member of the present invention is very suitable for ornaments for which a delicate color is required.

In the present invention, the aluminum alloy as constituting the substrate preferably has a limit upsetting ratio, at temperatures of from 200°C to 600°C, of 70% or more, and a tensile elongation, at room temperature, of 10% or more. This makes it possible to obtain a complicated shape easily by hot-working one or two times at a temperature of from 200°C to 600°C.

If a complicated shape is obtained by hot-working one or two times at from 200°C to 600°C in the case where the limit upsetting ratio is less than 70% or the tensile elongation at room temperature is less than 10%, work-cracks are generated.

The limit upsetting ratio is an upsetting ratio at which, when a hot-solidified body is upset at a forging rate of 0.5 mm/second, an edge portion of the solidified body begins to crack. The upsetting ratio is represented by ${\text{(L}}_{\text{0}} {\text{-L}}_{\text{1}} {\text{)/L}}_{\text{0}} \text{× 100 (%)}$ where L₀ represents the length along the upsetting direction of a sample before upsetting, and L₁ represents the length along the upsetting direction of the sample after the upsetting.

In the present invention, it is preferable that in the metal texture of the aluminum alloy constituting the substrate, the average grain size of aluminum crystals is 500 nm or less and the average grain size of an intermetallic compound is 300 mm or less. This makes it possible to set the hardness HRB of the substrate at from 50 to 100, and makes forging (molding) ability good.

If the average grain size of the aluminum crystals is over 500 nm or the average grain size of the intermetallic compound is over 300 nm, the ductility and the limit upsetting ratio of the aluminum alloy are improved, but the hardness decreases.

In the present invention, the ornamental aluminum alloy member is preferably an exterior part for watches, an ornament, or a part for electric equipment, or household electrical appliances.

A process for producing an ornamental aluminum alloy member, according to the present invention, comprises the steps of: (a) forming a molded body made of an aluminum alloy containing from 0.1% to 3% by weight of Zr, from 0.1% to 15% by weight of Mm, from 0.1% to 5% by weight of Mg, and the balance of Al; (b) heating the molded body to a temperature of from 200°C to 600°C under the condition of a temperature-raising rate of 2°C/second or more; (c) working the heated molded body, and (d) subjecting the worked molded body to anodic oxidation treatment.

According to the present invention, the aluminum alloy having the above-mentioned composition is used so that it is possible to mold the aluminum alloy with good moldability, obtain high hardness and make the color tone of the anodic oxidation film light.

If the temperature for heating the molded body is over 600°C or the temperature-raising rate is less than 2°C/second, in the texture of the aluminum alloy after the hot-working, its aluminum crystal grains or its intermetallic compound grow large so that its hardness decreases. If the temperature for heating the molded body is less than 200°C, the adhering of rapidly solidified powders to each other becomes insufficient and the aluminum alloy becomes brittle, resulting in that the limit upsetting ratio in the range of 200 to 600°C and the tensile elongation at room temperature decrease. The molded body is usually heated to that temperature from room temperature.

In order to obtain better property, the temperature for heating the molded body preferably ranges from 350 to 450°C. The temperature of a mold used in this case is preferably 400°C.

In the process of the invention, the step (a) preferably comprises a step of molding rapidly solidified powder of the aluminum alloy. This makes it possible to make the grain sizes of the aluminum crystal and the intermetallic compound fine in the texture of the aluminum alloy.

In the process of the invention, the step (c) preferably comprises a step of hot-working the heated molded body into a solidified powder, and subsequently warm- or hot-working the solidified powder. This makes it possible to obtain a complicated shape easily by working one or two times.

In the process of the invention, the molded body is preferably formed so as to have a shape of a rod or a plate. This makes it possible to select the shape of the molded body appropriately.

In the process of the invention, the step (b) preferably comprises a step of heating the molded body by induction heating, with the time for heating the molded body being within one minute. This makes it possible to suppress the growth of the crystal grains in the texture of the aluminum alloy.

In the process of the invention, it is preferable that the working applied to the heated molded body during the step (c) is warm- or hot-molding, and the number of molding times is 2 or less.

The composition of the aluminum alloy of the invention makes it possible to work the aluminum alloy into a complicated shape even by working one or two times.

In the process of the invention, the above-mentioned 2-time moldings preferably has a first molding of making an external shape of the molded body into a substantially final shape and a second molding of molding the surface of the molded body shallowly. This makes it possible to give the aluminum alloy a shape and to ornament it with letters, patterns or the like by a small number of molding times.

In the process of the invention, it is preferable that the working applied to the heated molded body during the step (c) consists of a first molding of making an external shape of the molded body into a substantially final shape and a second molding of molding the surface of the molded body shallowly, and the first molding is warm- or hot-molding and the second molding is cold-molding. Thus, it become possible to give the aluminum alloy a shape and ornament it with letters, patterns or the like by a small number of molding times.

In the process of the invention, it is preferable that the step (d) includes a sealing treatment, and as the sealing treatment, a pressurized steam sealing process or a nickel acetate sealing process is used. By this sealing treatment, the corrosion resistance of the anodic oxidation film can be improved.

In the process of the invention, it is preferable that the step (d) includes coloring treatment, and as the color treatment, a dyeing process, naturally color-developing process or an electrolytic coloring process is used. This coloring treatment makes it possible to color the anodic oxidation film.

Referring to the attached drawings, the present invention will be described by way of embodiments thereof hereinafter.

FIG. 1 is a partial cross sectional view of a wrist watch case 10, as an example of the ornamental aluminum alloy member according to the present invention. The wrist watch case 10 has a body 1 composed of a substrate or a molded body made of an aluminum alloy, and an anodic oxidation film 2 with which the whole surface of the body 1 is covered.

The aluminum alloy constituting the body 1 has a composition containing from 0.1% to 3% by weight of Zr, from 0.1% to 15% by weight of Mm, from 0.1% to 5% by weight of Mg, and the balance of Al, as described above. The aluminum alloy constituting the body 1 preferably further contains from 0.1% to 5% by weight of at least one metal element selected from the group consisting of Mo, W, Nb, Ag and Ta, as described above.

The hardness HRB of this body 1 is from 50 to 100. The lightness (L*) of the anodic oxidation film 2 is 50 or more. The electric conductivity of the body 1 is preferably 20% IACS or more. The anodic oxidation film 2 is preferably transparent and colorless, off-white or silver white.

It is preferable for the body 1 that its limit upsetting ratio at a temperature of from 200 to 600°C is 70% or more and the tensile elongation at room temperature is 10% or more.

For the texture of the aluminum alloy constituting the body 1, it is preferable that the average grain size of aluminum crystal grains is 500 nm or less and the average grain size of an intermetallic compound is 300 nm or less.

The following will describe a process for producing the wrist watch case 10 as shown in FIG. 1.

FIGS. 2 to 9 illustrate the steps of the process for producing the wrist watch case in the order of these steps. First, referring to FIG. 2, there is prepared rapidly solidified powder of an aluminum alloy containing from 0.1% to 3% by weight of Zr, from 0.1% to 15% by weight of Mm, from 0.1% to 5% by weight of Mg, and the balance of Al. This rapidly solidified powder is extruded so as to form a rod or a plate made of the aluminum alloy. The rod or the plate is cut into suitable sizes so that a bullet 3 having a cylindrical shape is produced.

Referring to FIG. 3, there is used an induction heating coil 4 connected to a power source which can adjust a supplying electric power and supplying time, to heat the bullet 3 up to 460°C in a short period of time by induction heating. The applied induction frequency is 1 kHz. The short period of time herein is preferably within one minute. The input electric power is adjusted in the manner that the heating can be finished for, e.g., 10 seconds.

Referring to FIG. 4, the induction-heated bullet is supplied into a warm- or hot-molding mold composed of a punch 5 and a die 6, and then is pressed into a finally-molded shape of a wrist watch case by means of a friction press machine which can apply a pressure of 150 tons. In this way, a molded product 1 providing the body is produced. The press is performed only one time. The warm- or hot-molding mold has been heated to 200°C with a heater.

The aluminum alloy before this warm- or hot-molding has a metal texture in which the grain size of aluminum crystals is 500 nm or less and the grain size of a precipitated intermetallic compound is 300 nm or less. By plastic deformation at high temperature, therefore, the crystal grain boundary sliding occurs without deformation of these crystal grains. This causes the limit upsetting ratio at a temperature of from 200 to 600°C to be 70% or more. Accordingly, warm- or hot-molding as described above makes it possible to mold the aluminum alloy into a final shape of a wrist watch case by extrusion only one time.

Referring to FIG. 5, an excess 1A of the molded product 1 is cut in a deburring step.

Referring to FIG. 6, the molded product 1 is latched to make fitting portions 1a and 1b to which glass and movements to be equipped with the watch are to be fitted.

Referring to FIG. 7, the molded product 1 is worked to make a hole 1c for a winding crown, a push button or the like.

Referring to FIG. 8, in order to finish the surface of the wrist watch case well, a buffing machine 7 is used to buff up the surface. Since the aluminum alloy constituting the molded product 1 has a fine metal texture, sufficient surface-gloss can be obtained by relatively light buffing.

Referring to FIG. 9, the molded product 1 is washed with an organic solvent to remove fat. Subsequently, for gloss finishing, the molded product 1 is chemically-polished or electrolytically-polished. For satin finishing, the molded product 1 is subjected to a matting treatment with sodium hydroxide.

After the respective steps are finished, the molded product 1 is subjected to anodic oxidation to form an anodic oxidation film 2 on the whole surface of the molded product 1. This anodic oxidation is performed, for example, by forming the anodic oxidation film 2 having a thickness of 15 µm by electrolysis using a sulfuric acid method. In the sulfuric acid method, for example, 15% sulfuric acid is used as a bath composition and the following conditions are used. Bath temperature: 20°C, current density: 1.5 A/dm³, and electrolyzing time: 60 minutes. The anodic oxidation may be performed using oxalic acid instead of sulfuric acid. In this case, higher abrasion-resistance can be expected. However, the resultant film develops yellow. Thus, this oxalic acid treatment is convenient for products to be colored golden, but cannot be used for products to be colored other colors.

In the case where conventional molten aluminum alloy is used, exterior parts for watches are frequently subjected to low-temperature anodic oxidation, that is, so-called herdamite treatment, in order to harden its surface and improve abrasion-resistance. In the present invention, however, it is desirable to perform anodic oxidation using the usual sulfuric acid method (treating temperature: 20°C). In the present invention, the aluminum alloy has a fine metal texture as described above so that the aluminum alloy has high strength, hardness and toughness at ambient temperature. For this reason, even if a low-temperature anodic oxidation film, that is, herdamite film is not used, the aluminum alloy can be satisfactorily used as exterior parts for watches in the present invention.

In the exterior parts for watches using a conventional molten aluminum alloy subjected to low-temperature anodic oxidation treatment, that is, so-called herdamite treatment, the thickness of the oxide film resulting from the treatment is at most about 20 µm. Accordingly, such aluminum alloy is liable to be injured by external force. The present invention is advantageous against such a problem since the hardness of the aluminum alloy material itself is high. Of course, it is evident that if the aluminum alloy of the present invention is subjected to low-temperature anodic oxidation, the aluminum alloy can be made into further preferred favorite exterior parts for watches from the standpoint of strength.

The molded body 1 subjected to the anodic oxidation is optionally colored. For the coloring, a dyeing method, a naturally color-developing method or an electrolytic coloring method is available. For exterior parts for watches, a delicate color tone is frequently required since they are ornaments. On the other hand, weatherability such as ultraviolet ray resistance is also demanded. To realize the delicate color, the dyeing method is industrially optimal. However, some dyes are insufficient in weatherability, and in particular organic dyes are insufficient in weatherability. In this case, a dye having a color similar to a required color is selected from inorganic dyes, which have sufficient weatherability but have limited sorts of colors, to perform a first dyeing, and then in a second dying an appropriate dye is selected from organic dyes, which have many sorts of colors, to realize the required color. In this way, it is possible to minimize fading by ultraviolet rays.

Thereafter, the anodic oxidation film 2 is subjected to a sealing treatment to improve corrosion resistance. As this sealing treatment, there is used, for example, a pressurized steam sealing method or a nickel acetate sealing method. The pressurized steam sealing method is a treatment of washing the product, which has been subjected to the anodic oxidation, with water, putting the product into an autoclave, and keeping the product therein under water vapor (steam) pressure of 3-5 kg/cm² for 20-30 minutes so as to seal the pores in the anodized film. In the present embodiment, the product is kept in steam at a pressure of 0.5 MPa for 15 minutes to fill holes.

The nickel acetate sealing method is a treatment of immersing an anodic oxidation film in an aqueous solution of nickel acetate to seal the pores.

In the above-mentioned embodiment, the present invention has been described with reference to the wrist watch case 10 as an ornamental aluminum alloy member. The present invention should not, however, be limited to this embodiment, and may be applied to other exterior parts for a watch such as a band for a watch, a vessel and a back flap, ornaments such as a bracelet, a finger ring and a tiepin, parts for electronic equipment such as a notebook-size personal computer, parts for household electrical appliances, parts for vehicles such as an automobile and a train.

Incidentally, the heated bullet 3 as shown in FIG. 3 may be molded into a final product by only a first molding of molding the bullet 3 into a final shape, as shown in FIG. 4, and a second molding of molding the surface thereof shallowly. The second molding is for ornamenting the molded bullet 3 with letters, patterns or the like. In this case, the first molding, as described with reference to FIG. 4, is preferably warm- or hot-molding. The second molding may be cold-molding, or warm- or hot-molding.

The advantages of the present invention will be made clear by the following Examples of the present invention together with Comparative Examples.

### Examples

A gas atomizing device was used to produce aluminum alloy powders having alloy compositions shown in Table 1 below (Examples 1-14 and Comparative Example 1-10). For atomizing, nitrogen gas was pressurized to 100 kgf/cm² and bombarded onto the molten aluminum alloys that were fallen from a nozzle having a hole of 2 mm in diameter. Instead of nitrogen gas, inert gas such as argon may be used.

Under the same atomizing conditions as above, a powder of 2014 aluminum alloy was produced, and then an actual cooling rate was estimated by measuring intervals between dendrite arms (dendrite crystals) of the texture of the powder. As a result, in the case where a powder having a grain size of 150 µm was obtained, the cooling rate thereof was 1 × 10³°C/sec.

Next, powders having a size of less than 150 µm were separated with a sieve from the respective aluminum alloy powders produced as above. The respective aluminum alloy powders were press-molded, and then the molded bodies were heated to a temperature in the range of 350 to 550°C at a temperature-raising rate of 2°C/sec. or more, while effecting degassing. Thereafter, the molded bodies were inserted into molds at a temperature of 400°C, and then were solidified at a face pressure of 9 tons/cm². The textures and mechanical properties were examined for the solidified powders produced under the above-mentioned conditions.

The texture of the solidified powders was examined by high-resolution SEM photographs. The results demonstrate that in all of Examples 1 to 14 the average grain size of aluminum crystals was 500 nm or less and the average grain size of intermetallic compounds was 300 nm or less, as shown in Table 1.

In order to study the forgeability of these solidified powders, their limit upsetting ratios at 400°C were examined. The results demonstrate that all of Examples 1 to 14 had a limit upsetting ratio of 70% or more so as to exhibit excellent forging ability, as shown in Table 2 below.

The surfaces of the solidified powders were machined. Thereafter, the solidified powders were washed with caustic soda and then were anodized until the thickness of the resultant anodized film became 10 µm. The color tone and gloss of the anodized aluminum were examined. The results demonstrate that the colors of the anodized aluminum films (anodic oxidation films) in all of Examples 1 to 14 were light, i.e., silver white, off-white, light yellow or light gray, as shown in Table 2. The films were also glossy.

The texture in the vicinity of the boundary between the anodized aluminum film and the substrate phase was examined by high-resolution SEM photographs. It was found from reflection electron images of this texture that an intermetallic compound was present in the anodized aluminum film, but in a small amount. That is, it was made clear that if the amount of the intermetallic compound in the anodized aluminum film is small, the color tone of the anodized aluminum film becomes a light color such as silver white or off-white. It was also made clear that in order to realize a light color, the area percentage of the intermetallic compound per unit area must be 20% or less.

Correlative relationship was examined between the electric conductivity of the substrates and the color tone of the anodized aluminum films. As a result, it was also made clear that when a light color such as silver white or off-white was obtained, the electric conductivity was 20% IACS or more, as shown in Table 2. Correlative relationship was examined between the color tone of the anodized aluminum films and lightness (L*). As a result, it was also made clear that in order to realize a light color, the lightness (L*) of the anodized aluminum films was 50 or more, as shown in Table 2.

In all of Examples 1 to 14, the hardness HRB of their parent phases was from 50 to 100 at room temperature (20°C) and the tensile elongation was 10% or more at room temperature (20°C).

On the other hand, results of Comparative Examples are as follows.

Comparative Examples 1 and 3 are cases wherein the temperature-raising rate at the time of heating the molded body was lower than 2°C/sec., and the heating temperature was higher than 600°C, respectively. In both the cases, in the textures of the solidified powders after the hot-working their aluminum crystal grains and intermetallic compounds grew large. Thus, their hardness was highly reduced.

In Comparative Example 2, the heating temperature of the molded body was lower than 200°C. In this case, the hardness became relatively high, but the color tone of the anodized aluminum film was dark.

In Comparative Example 4, the Zr content was more than 3% by weight. In this case, the intermetallic compound became fat and the precipitated amount thereof became large so that the hardness rose. However, the elongation at room temperature and the limit upsetting ratio at high temperature decreased. The remnant of the intermetallic compound was present in the anodized aluminum film subjected to the anodic oxidation. Thus, the color tone of the anodized aluminum film became dark.

In Comparative Example 5, the Mm content was more than 15% by weight. In this case, the intermetallic compound grew large and the precipitated amount thereof became large so that the hardness was increased. However, the elongation at room temperature and the limit upsetting ratio at high temperature decreased. The large amount of the intermetallic compound caused the remnant of the intermetallic compound to be present in the anodized aluminum film subjected to the anodic oxidation. Thus, the color tone of the anodized aluminum film became dark.

In Comparative Example 6, the Mg content was more than 5% by weight. In this case, the intermetallic compound grew large and the precipitated amount thereof became large so that the hardness was increased. However, the elongation at room temperature and the limit upsetting ratio at high temperature decreased. The large amount of the intermetallic compound caused the remnant of the intermetallic compound to be present in the anodized aluminum film subjected to the anodic oxidation. Thus, the color tone of the anodized aluminum film became dark.

In Comparative Examples 7 to 9, Mo or W was contained in an amount of more than 5% by weight. In these cases, the color tone of the anodized aluminum film also became dark.

In Comparative Example 10, Zr was contained in an amount of less than 0.1% by weight. In this case, aluminum crystal grains grew large so that the hardness decreased.

As described above, in Examples 1 to 14, there were used aluminum alloys having the composition shown in Table 1 (Zr: from 0.1% to 3% by weight; Mm: from 0.1% to 15% by weight; Mg: from 0.1% to 5% by weight; and the balance: Al) and conditions for heating the molded bodies shown in Table 1 (heating temperature: 200°C or more, but 600°C or less; and temperature-raising rate: 2°C/sec. or more). Therefore, it was possible to obtain aluminum alloys for ornament having high hardness, a light-colored anodized aluminum film, and good moldability.

As has been described above, the ornamental aluminum alloy member of the present invention can be easily molded into a complicated shape. Its substrate has a high hardness, and its anodized film became light in color.

The embodiments and Examples disclosed in the above are illustrative and are not restrictive. The scope of the present invention should not be limited to the above disclosure and should be defined by the claims. The present invention includes all modifications and equivalents to the claims.

## Claims

1. An ornamental aluminum alloy member, characterized by comprising:
a substrate made of an aluminum alloy comprising from 0.1% to 3% by weight of Zr, from 0.1% to 15% by weight of Mm, from 0.1% to 5% by weight of Mg, and the balance of Al; and
an anodic oxidation film formed on a surface of the substrate.

2. The ornamental aluminum alloy member, characterized comprising a substrate formed of an aluminum alloy, and an anodic oxidation film formed on a surface of the substrate,
wherein said substrate has a hardness HRB of from 50 to 100, and said anodic oxidation film has a lightness of 50 or more.

3. The ornamental aluminum alloy member according to claim 1 or 2, characterized in that said substrate further contains from 0.1% to 5% by weight of at least one metal element selected from the group consisting of Mo, W, Nb, Ag and Ta.

4. The ornamental aluminum alloy member according to claim 1 or 2, characterized in that said substrates has an electrical conductivity of 20% IACS or more.

5. The ornamental aluminum alloy member according to any one of claims 1 to 4, characterized in that said anodic oxidation film is transparent and colorless, off-white or silver white.

6. The ornamental aluminum alloy member according to any one of claims 1 to 5, characterized in that said aluminum alloy constituting the substrate has a limit upsetting ratio of 70% or more at temperatures of from 200°C to 600°C, and a tensile elongation of 10% or more at 20°C.

7. The ornamental aluminum alloy member according to any one of claims 1 to 6, characterized in that the metal texture of said aluminum alloy comprises aluminum crystals and intermetallic compounds, and the average grain size of the aluminum crystals is 500 nm or less and the average grain size of the intermetallic compounds is 300 nm or less.

8. The ornamental aluminum alloy member according to any one of claims 1 to 7, which is an exterior part for watches, an ornament, or a part for electronic equipments or household electrical appliances.

9. A process for producing an ornamental aluminum alloy member, characterized by comprising the steps of:
(a) forming a molded body made of an aluminum alloy containing from 0.1% to 3% by weight of Zr, from 0.1% to 15% by weight of Mm, from 0.1% to 5% by weight of Mg, and the balance of Al;
(b) heating the molded body up to a temperature of from 200°C to 600°C under the condition of a temperature-raising rate of 2°C/second or more;
(c) working the heated molded body; and
(d) subjecting the worked molded body to anodic oxidation treatment.

10. The process according to claim 9, characterized in that said step (a) comprises a step of molding rapidly solidified powder of said aluminum alloy.

11. The process according to claim 9 or 10, characterized in that said step (c) comprises a step of hot-working the heated molded body into solidified powder, and subsequently warm- or hot-working the solidified powder.

12. The process according to any one of claims 9 to 11, characterized in that said molded body is formed so as to have a shape of a rod or a plate.

13. The process according to any one of claims 9 to 12, characterized in that said step (b) comprises a step of heating the molded body by induction heating, with the time for heating the molded body being within one minute.

14. The process according to any one of claims 9 to 13, characterized in that said working applied to the heated molded body is warm- or hot-molding, with the number of molding times is 2 or less.

15. The process according to any one of claims 9 to 14, characterized in that 2-time moldings has a first molding of making an external shape of the molded body into a substantially final shape, and a second molding of molding the surface of the molded body shallowly.

16. The process according to any one of claims 9 to 13, characterized in that said working applied to the heated molded body consists of a first molding of making an external shape of the molded body into a substantially final shape, and a second molding of molding the surface of the molded body shallowly,
said first molding is warm- or hot-molding and said second molding is cold-molding.

17. The process according to any one of claims 9 to 16, characterized in that said step (d) includes a sealing treatment, and as the sealing treatment a pressurized steam sealing process or a nickel acetate sealing process is used.

18. The process according to any one of claims 9 to 17, characterized in that said step (d) includes coloring treatment, and as the color treatment a dyeing process, naturally color-developing process or an electrolytic coloring process is used.
